

Aug. 28, 1923.

1,466,627

K. P. McELROY

PROCESS OF MAKING CYANIDS

Filed Jan. 25, 1922

2 Sheets-Sheet 1



*INVENTOR*  
K. P. McElroy.

Aug. 28, 1923.

1,466,627

K. P. McELROY

PROCESS OF MAKING CYANIDS

Filed Jan. 25, 1922

2 Sheets-Sheet 2



## UNITED STATES PATENT OFFICE.

KARL P. McELROY, OF WASHINGTON, DISTRICT OF COLUMBIA, ASSIGNOR TO FERRO CHEMICALS INC., OF WASHINGTON, DISTRICT OF COLUMBIA, A CORPORATION OF DELAWARE.

## PROCESS OF MAKING CYANIDS.

Application filed January 25, 1922. Serial No. 531,614.

To all whom it may concern:

Be it known that I, KARL POMERY McELROY, a citizen of the United States, residing at Washington, in the District of Columbia, have invented certain new and useful Improvements in Processes of Making Cyanids, of which the following is a specification.

This invention relates to processes of making cyanids; and it comprises a method wherein cyanid forming materials are fed to a suitable reaction chamber in which a dominant mass or pool of cyanid in the liquid and the vapor phase is maintained by aid of heat supplied by electrical means, the temperature being maintained above 1000° C. and cyanid being removed and recovered from the sphere of reaction as liquid or as vapor; all as more fully hereinafter set forth and as claimed.

20 The present invention is in part based upon a discovery that at temperatures above 1000° C. cyanid reacts with oxidized forms of alkali to form carbon monoxid, setting free nitrogen and alkali metal and that in making cyanid, the initial presence of cyanid itself in substantial proportions accelerates the conversion of alkali to cyanid in the presence of carbon and nitrogen. I have found that in systems comprising alkali, cyanid, carbon, nitrogen and carbon monoxid the conversion of alkali to cyanid is accomplished with what may be termed commercial velocity when the alkali and cyanid are present as vapor in substantial concentrations in the gas phase of the system, that is, at temperatures ranging above 1000° C. at about one or two atmospheres pressure.

40 Alkali, carbon and nitrogen when heated together form cyanid. The reaction is highly endothermic and most of attempts which have been made to utilize it technically have failed because of the inherent difficulty of supplying heat for the reaction through retort walls externally heated. Attempts to supply heat by electrical means have likewise failed because of lack of means for temperature control, and because there was no adequate means of proportioning the load of work to be done to the supply of energy available for the cyanid forming reaction. Another cause for lack of success has been failure to allow

for the tendency of cyanid to revert to alkali in presence of CO at temperatures below those at which cyanid is formed.

55 In a copending application Serial No. 477,205, filed June 13, 1921, I have described and claimed a process of making cyanid from alkali, carbon and atmospheric nitrogen wherein these materials are heated together to a temperature well over 1000° C. in a blast furnace such as is used for making pig iron, the operation of the furnace being so regulated that a dominant mass or pool 60 of cyanid liquid and vapor is maintained in the hot zone of the furnace, the alkali being fed to such pool and cyanid removed therefrom at a rate proportioned to the supply of heat thereto. In the invention which 65 is the subject matter of said application the source of heat used is the combustion of preheated carbon under gas producing conditions (that is to carbon monoxid) with preheated air, said combustion taking place 70 in or in proximity to said dominant pool of cyanid. In said application the reinforcement of the combustion heat by electrically developed heat is described but not claimed. It is an object of the present invention to 75 so utilize electrical heat and proportion the supply of electrically developed heat relative to the combustion heat that a very high concentration of cyanid vapor is possible 80 in the gases produced; the cyanid producing 85 capacity of a furnace of given size being substantially increased over that which is possible when gasification of carbon with air constitutes the main supply of heat.

90 Since sodium cyanid is now the standard commercial form of cyanid and since sodium carbonate (soda ash) on account of its cheapness and its composition is an advantageous source of alkali for making cyanid, I shall describe the invention with particular reference to making sodium cyanid from sodium carbonate, it being understood 95 that the invention is applicable to the production of any other cyanid. I may use as the alkali of the process the oxid or carbonate (or compound capable of yielding these), of any alkali or alkaline earth or even the alkali or alkali earth metals themselves and produce the corresponding metal cyanid. For example potash, baryta, strontia, lithia 100 or even thallia are available in this connec- 105

tion. Lime or magnesia however is more advantageous in admixture with other alkalis than alone.

The formation of cyanid from sodium carbonate, carbon and nitrogen may be represented by the reversible reaction:—



The chemical energy involved in this reaction is, according to generally accepted data on heats of formation, 134320 calories, plus or minus. This quantity of heat is absorbed in the formation of cyanid from carbonate or is set free in the reversal of the reaction. The reaction comes to an equilibrium with a ratio of cyanid to carbonate depending partly upon the relative concentrations in the system of nitrogen and carbon monoxid and partly upon the temperature. Above 1200° C. cyanid is practically 100 per cent stable in the presence of CO alone and the conversion of carbonate to cyanid, with substantial proportions of initially present cyanid, takes place quickly and completely. From the practical standpoint therefore, the production of cyanid becomes a matter of an adequate supply of heat available for the reaction at a temperature around 1200° C. Since at these temperatures the vapor pressure of cyanid is quite large the cyanid formed is to a great extent in the vapor phase and heat for vaporization is required in addition to the heat of reaction. The total work of converting carbonate, carbon and nitrogen to cyanid vapor at 1200° may be estimated to be, (per molecule NaCN):

|                                             | Calories. |
|---------------------------------------------|-----------|
| Heat absorbed in reaction-----              | 67160     |
| Sensible heat of NaCN at 1200°-----         | 23000     |
| Latent heat of fusion and vaporization----- | 34500     |
| Sensible heat 1½ molecules CO-----          | 13400     |
|                                             | 138060    |

The semi-combustion of carbon to form carbon monoxid evolves only about 30 per cent of the total heat of combustion of carbon but this amount is sufficient to raise all of the products of combustion to 1200° C. and leave a margin over available for making cyanid; that is for heating a certain further amount of carbon up to this temperature and producing cyanid from it. The greater the preheat which can be given air and carbon the greater is this margin; and contra, the greater the heat losses by radiation and the like, the less the margin. Radiation losses are proportional to temperature, time and area of exposed surface, and the faster the semi-combustion can be driven and the larger the furnace unit, the less the percentage loss of heat in this way. In large apparatus like a blast furnace or

a big gas producer, using preheated blast and preheated fuel (see application Serial No. 477,205) the gasification of carbon with air may theoretically be as low as 0.3 to 0.5 pound per pound of cyanid produced in the gases in the vapor form. With lower temperatures giving slower reaction and with smaller apparatus, the figures are not so favorable.

In the yield just mentioned, the cyanid is in the vapor form and this represents an expenditure of heat which, if the cyanid were delivered as liquid, would be available for the production of more cyanid. In the production of cyanid by semi-combustion of carbon with air as a source of heat, of necessity a large volume of gases is produced; this gas being carbon monoxid from the carbon and from the alkali carbonate and unused nitrogen. As sodium cyanid has a high vapor tension at 1200°, with this bulk of gases the product exists in the vapor form. With a less volume of gases, more or less of it occurs in the liquid form with a concomitant decrease in the amount of heat needed for cyanidation.

In one embodiment of the present invention I maintain a high concentration of cyanid vapor in the gases produced in the hearth or combustion zone of a blast furnace or slagging gas producer by reinforcing the combustion heat by heat electrically developed in said zone. At the same time I so proportion the feed of alkali to the furnace and the withdrawal of gases at a low point in the furnace to the supply of heat to said hot zone that a dominant pool of cyanid, as liquid and vapor, is established and maintained therein, as more fully described in my application Serial No. 477,205. In so doing, the production of cyanid is smooth and regular and the capacity of a given furnace is increased over that which is possible when combustion heat alone is used. Furthermore in working thus, the production of cyanid in a relatively small sized furnace becomes profitable whereas in very small furnaces, using combustion heat alone, the radiation and cooling factor is of such weight that the concentration of cyanid vapor in the gases may be small and the time yield concomitantly low. The proportion of combustion heat to electric heat may be as desired. I usually find it advantageous, on account of the relative costs of combustion heat and electric energy, to have the proportion of combustion heat large and to apply electric energy in quantity sufficient merely to overcome heat losses, thereby maintaining a high concentration of cyanid vapor without unduly fast driving. But I may in some cases rely principally upon electrical heating and make the combustion heat of subordinate weight, merely passing air into the reaction zone at a rate sufficient to maintain

an excess of nitrogen therein. In one embodiment of the invention hereinafter described, I may use electrical heat alone and I may even pass nitrogen instead of air or mixed 5 with air into the reaction zone. In this embodiment part of the cyanid is removed from the reaction zone in the liquid state, the use of electric heat serving to keep the volume of gases, and thereby the vaporization of 10 cyanid, at a minimum.

In recovering cyanid from gases carrying it by condensing the vapor and depositing fume it is desirable to quickly cool such gases so as to pass rapidly through the 15 temperature range at which cyanid tends to revert to alkali in the presence of CO and in this connection it makes for economy to have the concentration of cyanid vapor high and that of other gases low. When using 20 electrical heat as above described, the temperature of the reaction zone may be controlled independently of the speed of gas flow. The predominance of cyanid in the 25 reaction zone is secured by this temperature control which results from proportioning the input of electric energy to the feed of cyanid forming materials going to the reaction zone and the withdrawal of cyanid and heated gases therefrom. The 30 temperature is advantageously above 1000° C. and it is advantageous to keep it about 1200°. In using fuels with high ash as a source of carbon it is advisable to run at an ash-slagging 35 temperature with addition of lime, or other suitable flux, and the temperature may then be from 1400° to 1500°; the gases may in this case be taken from the reaction chamber at lower temperatures.

The application of electric heat to the 40 cyanid forming reaction zone is accomplished by any suitable or convenient means. In a shaft furnace provided with tuyères near the bottom for blowing with hot air and with outlets for hot gases above the 45 bosh or fusion zone, current may be supplied to the hot zone by means of electrodes placed in suitable apertures through the furnace walls, the furnace charge, comprising charcoal or coke impregnated with cyanid 50 and alkali serving as resistance material. Or the slag bath in the bottom of the furnace may be used as resistor, heat electrically generated therein radiating upwardly to the reaction zone. Or an electric furnace 55 of the arc type with multiphase currents may be used, such furnace being provided with tuyères for admission of hot air and having a superimposed shaft through which a regulated proportion of the cyanid laden 60 gases from the hot zone passes upward in counter-current to a descending charge of alkalinized fuel, and cyanid being condensed and recovered from a portion of said gases which are led from the furnace while they 65 are at a temperature above 1000° and quick-

ly cooled or otherwise treated for the separation of cyanid. A convenient method for supplying electric heat is by means of eddy currents induced in suitably prepared conducting linings provided in the hot zone, 70 this zone being surrounded by heat insulating material and, outside of this, by a coiled electric conductor carrying high frequency alternating current. This method of applying electric heat is of particular advantage 75 with a small slagging gas producer where it may be desirable merely to compensate losses by electrically developed heat and where the heat of gasification of preheated carbon with preheated air may be relied 80 upon for the greater proportion of the necessary heat supply to the hot zone. The induction method may however also be conveniently utilized in a shaft furnace where electric energy is the main source of heat, that is, where combustion heat is only incidental and considered merely as lessening the heat requirement of the cyanid reaction. It may here be noted that the use of air is usually preferable to that of nitrogen alone and that 85 enrichment of the air with oxygen also makes for energy economy.

In the drawings annexed hereto I have shown, more or less diagrammatically, certain apparatus elements within the present 90 invention and adapted for use in the operation of the described method.

Fig. 1 is a view in central vertical section of an induction furnace;

Fig. 2 is a similar view of a resistance 100 furnace;

Fig. 3 is a similar view of an arc-heated furnace and

Fig. 4 is a detail of a condensing arrangement.

Fig. 1 shows an electric induction furnace in which near the top, as shown, is a bustle pipe 1 fitted with tuyères for carrying air into the furnace. Element 2 is a gas outlet near the bottom, 3 a hole for drawing off molten cyanid, and 4 is a cylinder forming the lining of the furnace. This is made of electric conducting material such as nichrome or other suitable refractory metal or it may be of graphitized carbon impregnated and coated internally with magnesia or other suitable material. 5 represents a water cooled electrical conductor with electrical leads 6 carrying high frequency alternating currents by means of which heating 110 currents are induced in the carbon cylinder 4 and in the alkalinized and cyanized carbon which is in the furnace. The furnace is charged with material at the top by means of the charging hopper and bell 7. The cylinder 4 is heat insulated by the material 8 consisting preferably of lamp black which is held in place by the casing 9 made of micanite or other electrical insulator. As shown, the bottom of the cylinder is inclined 120 125 130

downwardly from the gas outlet toward the cyanid hole 3.

Fig. 2 depicts an electric resistance furnace in which the charge of alkalinized and cyanized carbon constitutes the resistor. Elements 10 are air inlets, 11 the gas outlets, 12 the outlet for removal of molten material and 13 is a small carbon rod for carrying the starting current between the electrodes 14, supplied with current through electrical leads 15. The furnace is fed with alkali and carbon through the charging devices 16 provided, as shown, with bells and hoppers. The furnace as shown is built with a flare or increasing cross sectional area toward the bottom so as to decrease the electrical resistance of this part of the charge and concentrate the heating effect of the current toward the top. The casing 17 may be made of magnesite or chromite brick work or of other suitable material. The conduit 18 carries cyanid laden gases to apparatus for recovery of cyanid, which may be such as that shown in Fig. 4.

Fig. 3 shows a furnace of the blast furnace type provided with bustle pipe and tuyeres 20 as air inlet, hot gas outlets 21, metal and slag outlet 22, and cool gas outlet 23 near the top. Inserted in the bosh walls through water cooled openings are electrodes 24 with electrical leads 25. The furnace has the usual charging device 26. The hot gas outlets 21 lead into an annular conduit 27 which is connected by conduits 28 to apparatus for cyanid recovery, here shown as comprising a water jacketed condenser 29 containing cooling pipes 30. This is a type of apparatus adapted for quickly cooling the hot cyanid laden gases through the temperature range below 1000°, in which cyanid in presence of CO tends to revert to oxid and carbonate. Valves 31 and 32 are for the purpose of regulating the relative proportions of the furnace gases leaving the furnace through hot gas outlets 21 and passing up through the shaft and out by cold gas outlet 23.

Figure 4 shows another type of apparatus for quickly cooling cyanid laden gases; which may be used in connection with any of the furnaces herein described, being for example connected by inlet 35 to outlet 28 of the structure of Fig. 3 to outlet 18 of Fig. 2 or outlet 2 of Fig. 1. In this showing, inlet 35 is a conduit leading from the hot gas outlet of any cyanid furnace. Elements 36 and 37 are sheet metal towers connected at the bottom by conduit 38 and connected at the top by conduit 39. Conduit 38 is in the form of a hopper with a U-shaped bottom. In tower 37 are shown cooling pipes 40 in which air, water or other cooling medium circulates. Through the conduit 38 runs the conveyor 41 delivering into receptacle 42. A thermal circulation of gases may be main-

tained through the two towers by means of the cooling action of pipes 40, gas passing from 36 to 37 through 39 and from 37 to 36 through 38. There is thus maintained in 36 a mass of cold gas into which hot cyanid laden gas is delivered through 35 which may enter tangentially and downwardly. The hot gas is cooled quickly by admixture with the relatively large mass of cold gas in 36 and the heat thus admitted aids the gas circulation upwardly in 36 and downwardly in 37. Cyanid is quickly condensed in 36, falls to the bottom and is removed by conveyor 38. As condensation is favored by nuclei, dustlike suspended particles are built up until they are large enough to fall freely. The apparatus therefore gives or may be made to give, a granular product. Excess of gas passes out through pipe 43. Control of the volume of gas passing out of the apparatus and, therefore, of the volume of hot gas entering, is secured by adjustment of valve 44. A pyrometer 45 indicates the temperature resulting from the mixture of incoming hot gas with the mass of gas maintained in 36. The mass of hot gas which an apparatus of this type can handle is a matter of design. Usually the circulation through the towers is sufficiently rapid without the aid of a fan in conduit 39, but such a fan (not shown) may be used. There may be as many of these coolers connected to the hot gas outlet of a furnace as are required to handle the volume of hot gas required to be taken from the furnace in securing the desired regulation thereof as described.

The apparatus of Figs. 1 and 2 are worked similarly. They differ mainly in the means provided for applying electric energy. Being filled with alkalinized carbon in lumps (which may be charcoal, coke or other form of carbon impregnated with soda) the electric current is applied and the furnace brought up to about 1100°. Heated air is now blown or sucked in through 1 or 10 slowly at first and until the alkali in the furnace toward the bottom is practically completely cyanided. Cyanid may be used instead of carbonate for impregnating the carbon in starting. When the alkali in the furnace is cyanided, which can be tested by withdrawing a sample through 3 or 12, the air volume is increased and the feed of alkalinized carbon through 7 or 16 is correlated with the air volume, both being properly proportioned with regard to the electric energy applied, thereby maintaining the temperature at the desired degree. The gases leaving the furnace through 2 or 11 now carry cyanid vapor in concentrations (below the saturation point) depending upon the ratio between the electric energy applied and the heat of combustion. The latter is a function of the speed of driving (the volume of air per minute with the correlated alkali

and carbon feed). With the speed of driving fixed the concentration of cyanid vapor in the gases varies directly with the electric power (the rate of delivery of electric energy) and this may be sufficient to saturate the gases in the furnace with cyanid vapor at the temperature maintained. The excess of alkali fed over that sufficient to saturate the gas as it leaves the furnace collects as cyanid 5 in the molten state at the bottom of the furnace and is drawn off from time to time through 3 or 12. The collection of liquid cyanid in this way is aided by the flare of the furnace shown in Figure 2 and by placing 10 the induction coil 5 on the furnace of Fig. 1 well above the bottom, thus providing for a cooling effect and causing a condensation of cyanid from the gases before they leave the furnace. It is advisable with this type 15 of furnace to keep the temperature at a minimum consistent with adequate speed of cyanid formation, thus minimizing heat consumption and recovering in the molten state as described the maximum proportion of the 20 cyanid formed in the furnace.

In the operation as above described I am in effect continuously gasifying carbon by sodium carbonate and by air, maintaining a temperature at which soda is vaporized and, 25 in mixture with nitrogen and carbon monoxid, the soda vapor is contacted with carbon thereby forming cyanid, the conversion being accelerated by maintaining in the reaction zone substantial quantities of pre-formed cyanid serving as a dominant pool. With sufficiently fast driving, carbon dioxide 30 may be first formed in the upper zones of the furnace, the heat of  $\text{CO}_2$  formation being partially absorbed in vaporization of soda; the soda vapor and  $\text{CO}_2$  together with 35 nitrogen, all at a very high temperature, subsequently contact with carbon to form cyanid and  $\text{CO}$  with a drop in temperature as the gases proceed through the reaction zone.

40 The size of this zone should be greater, the greater the speed of driving. The proportions of alkali and carbon to be used in the alkalinized carbon fed to the furnace depend upon the ratio of electric heat to combustion heat, that is, upon the relative proportions of the carbon charged which are to be gasified by air and by soda. With nitrogen alone, carbon would be consumed only in the cyaniding reaction, the theoretical ratio 45 of carbon to sodium cyanid being 48 to 98 or 0.49 to 1. The ratio is equivalent to 2.2 parts sodium carbonate to one of carbon or, for example, about 66 parts soda ash to 34 parts of charcoal of 90 per cent carbon. When 50 using nitrogen alone heat would be supplied by electric power alone and the theoretical energy consumption may be estimated as about 1.5 kilowatt hours per pound of sodium cyanid vapor. The maximum concentration 55 of cyanid vapor, corresponding to

100 per cent fixation of the nitrogen passed into the furnace, would be 40 per cent by volume, assuming the vapor molecule to be represented by the formula  $\text{NaCN}$ . Using air in 100 per cent excess, that is with a 50 per cent fixation of its nitrogen, if the air be preheated to  $750^\circ$  and the gases taken off at  $1200^\circ$ , the theoretical electric energy requirement, as estimated, would be reduced 70 by about 9 per cent, the proportions of soda and charcoal would be 60 : 40 and the equivalent maximum concentration of cyanid vapor in the gases 28 per cent. For that proportion of the cyanid removed from the furnace in the molten state an estimated saving of 75 20 per cent of the energy requirement is indicated. Relying entirely upon combustion heat for the cyanid reaction proper, using electric heat in proportion sufficient merely to balance heat losses, the consumption of carbon with air preheated to say  $750^\circ$  and with the alkalinized carbon fed cold to the furnace, would be about 2.5 lbs. per pound cyanid, the ratio of soda in the alkalinized carbon would be 28 parts to 72 of charcoal of 80 85 90 95 100 105 110 115 120 125 130 90 per cent carbon and the cyanid would be in a volume concentration of about 4 per cent in the gases. Something over 3 per cent of the air nitrogen would be fixed as cyanid at the expense of 34 per cent of the calorific value of the carbon used. In this case it may be said that 80 per cent of the carbon is gasified by air and 20 per cent by soda. It will be seen from the foregoing that the procedure may be widely varied as desired to meet varying conditions as to power costs, fuel prices, scale of production, capital investment, demand for producer gas, etc. As heretofore noted, with an apparatus of given size or a fixed rate of gas flow, electric heating makes for a maximum time-yield and this tends to reduce all elements of overhead cost to a minimum.

Furnaces of the types shown in Figs. 1 and 2 may be operated discontinuously or batchwise. In batch operation, such a furnace may be charged with a mixture comprising carbon and alkali (alkalinized charcoal works well) and, brought up to about  $1000^\circ$  or above by electric heat. Air or nitrogen, (preferably preheated) is then passed into the furnace and alkalinized charcoal fed to the furnace at the same time, the proportion of alkali with the carbon being such, relative to the rate of gas flow, that alkali is fed and cyanid formed faster than the latter is removed from the furnace as vapor in the gases produced. As a result, cyanid accumulates in the furnace and the proportion of cyanid to residual charcoal may be brought to any desired concentration and the operation then discontinued. The furnace may then be cooled and the cyanized charcoal may be removed and utilized as such, or the cyanid may be separated

from the charcoal by suitable means such as leaching. Or the cyanid may be distilled or sublimed away from the furnace while the latter is still hot either under vacuum or by means of a circulating current of inert gas such as nitrogen, cyanid being deposited by cooling the efflux gases. Usually the continuous method of operation is preferable.

At about 1000° the vapor tensions of most alkalies and their cyanids is fairly small so that with a moderate feed of air or nitrogen (or air enriched in oxygen), a batch of alkalized charcoal in granular or lump form may be readily converted into cyanized carbon with a relatively small removal of cyanid or alkali in vapor form. With some alkalies, such as baryta, the temperature at which this is done can be higher than with potash or soda. The cyanized carbon will always contain some unconverted alkali; the amount depending upon temperature conditions. Carbon being consumed in the reaction, the proportion of cyanid and alkali (taken together) in the cyanized product is or may be greater than the proportion of equivalent alkali in the initial alkalized charcoal. When using soda as alkali, the operation may be so managed as to yield cyanized charcoal containing a total alkali equivalent of from 40 to 80 per cent sodium cyanid. The proportion of cyanid (and alkali) in the product depends upon the masses of nitrogen and oxygen relative to those of the carbon and alkali. By regulation of these proportions the said proportion of cyanid may be as desired.

The operation of the furnaces shown in Figs. 1 and 2 may be reversed by introducing air or nitrogen at the bottom and taking away gases at the top; air inlets and gas outlets being simply reversed in function. In this event, the operation may then be so managed that all or any part of the cyanid formed is removed from the furnace in the vapor state and recovered from the gases. When using air, furnaces of the types of Figs. 1 and 2 may be operated in a manner similar to the operation of the structure shown in Fig. 3.

In operating the furnace of Fig. 3, charcoal, coke, coal or other carbonaceous matter, impregnated or mixed with soda together with flux for slagging the fuel ash are charged into the furnace through 26. The furnace being filled and the charge ignited, the materials descend slowly in countercurrent to a regulated portion of ascending gases produced in the hearth by the gasification of so preheated carbon with preheated air introduced through 20. Gases produced in the furnace are withdrawn through outlets 21 and 23 in relative proportions definitely controlled in accordance with the furnace work; this control being effected by means of valves 31 or 44 and 32. Means

for causing the flow of gas through the furnace are not shown but may be either pressure applied to the inlet air line or differential suction applied to the respective outlet gas lines. The temperature in the hearth and combustion zone is kept very high, ranging from 2000° C. in the immediate vicinity of the tuyères to about 1200°, usually, at the level of the hot gas outlets 21. Electric heat is applied by means of current passing through the electrodes 24 placed, as shown, near the top of the bosh at opposite points on the circumference. Slag and metal if any be formed, are removed through 22 in usual ways. Cyanid is formed in the hot zone, passes upward as vapor with the gases and out of the furnace through 21, being recovered from the regulated portion of the furnace gases which is caused to flow through these outlets. The cyanid carried in the gas caused to pass up through the shaft is condensed, deposited and adsorbed in the descending alkalized carbon and the cyanid from the gas more or less reverts to oxid and carbonate in the cooler portion of the shaft. Thus the sensible heat of the CO and N<sub>2</sub> and also the latent heat of vaporization of cyanid, and to a greater or less extent the sensible heat and the energy of reversion of the cyanid to oxid and carbonate are applied to the preheating of the soda and carbon and to the work of cyanid formation, so that the shaft delivers to the combustion zone alkali and carbon, with the alkali already to a greater or less extent deoxidized or converted to cyanid and preheated. The proportion of the total work which is done in the shaft depends upon the regulation of the furnace operation, the principles of which may be illustrated as follows:—The work of converting cold carbonte, carbon and nitrogen to cyanid vapor and CO at 1200° has been hereinbefore estimated at 138060 calories per molecule NaCN. Under the countercurrent stated action in the shaft of the furnace, the sensible heat of the CO formed in the cyanid reaction is recuperated by the descending alkali and carbon and the item of 13400 calories per molecule NaCN estimated as the sensible heat of 1½ molecules CO at 1200° may be left out of the calculation, leaving the total heat required at 124660 calories per molecule NaCN or 2544 thermal units per pound cyanid. For purposes of illustration this work may be divided into three steps as follows:—

(1) Conversion of carbonate to oxid in the reaction, Na<sub>2</sub>CO<sub>3</sub>+C=Na<sub>2</sub>O+2CO, and preheating Na<sub>2</sub>O+3C to 1200°;

(2) Conversion at 1200° of liquid oxid to liquid cyanid in the reaction, Na<sub>2</sub>O+3C+N<sub>2</sub>=2NaCN+CO;

(3) Vaporization of liquid cyanid at 1200°.

The chemical energy involved in (1) may be taken as 114480 calories and in (2) as 130

19840 calories, making up the total chemical energy of 134320 calories or 67160 calories per molecule NaCN. With the molecular specific heat of 13 ( $1+0.00039 t$ ) the sensible heat of  $\text{Na}_2\text{O}$  at  $1200^\circ$  may be estimated as about 23000 calories; the molecular heat of fusion is estimated at 4500 calories; and the molecular figures may be taken as about the same for cyanid. The heat in carbon at  $1200^\circ$  is 5832 calories per gram-atom. Hence the work involved in the three steps may be estimated to be:

15 (1) 79238 calories per molecule or 1617 thermal units per pound cyanid.  
(2) 15422 calories per molecule or 315 thermal units per pound cyanid.  
(3) 30000 calories per molecule or 612 thermal units per pound cyanid.  
Total, 124660 2544 thermal units per pound cyanid.

The relative proportions of the gas from the combustion zone caused to leave the furnace through hot gas outlet (21) of Fig. 3, and top gas outlet (23) respectively may be so adjusted that any desired proportion of the work involved in steps (1) and (2) may be done in the shaft. It is usually economical so to manage the operation that electric energy is utilized in quantity only sufficient to compensate heat losses; and to cause sufficient gas carrying cyanid to pass up through the shaft in order to convert all descending alkali to liquid cyanid pre-heated to about  $1200^{\circ}$ ; in other words to complete steps (1) and (2) in the shaft leaving only step (3) or its equivalent to be done in the combustion zone. So working, carbon is needed in the hearth to be gasified with air at say  $750^{\circ}$  to the extent of about 0.32 pound per pound of vaporized cyanid. The corresponding volume concentration of cyanid vapor is about 20 per cent of the mixed gases. About 55 per cent of these gases, caused to pass up through the shaft where they contact with descending alkali and carbon, by virtue of their sensible heat and latent and potential energy developed in the condensation and partial cooling and reversion of cyanid and deposition of carbon is sufficient to complete the conversion to cyanid of sufficient alkali (which should be charged with the carbon) to replace the cyanid removed from the furnace in 45 per cent of the gases produced in the combustion zone. Such a proportion of said gases may be withdrawn through the hot gas outlets 21. The consumption of carbon in the gasification with air in the combustion zone is thus about 0.72 pound per pound of cyanid recovered from the 45 per cent of the gases and 0.49 pound carbon is consumed in the cyaniding reaction; but from the 55 per cent of the gas going up through the shaft carbon is deposited in the decomposition of CO and with full development in this way of the latent energy of CO from the combustion zone, the carbon so

deposited may amount to 0.2 pound per pound of recovered cyanid, leaving the net carbon requirement about one pound per pound of cyanid produced. The corresponding proportions of soda and carbonaceous fuel fed to the furnace are then about 50:50. 70

I may however withdraw hot and cool gas in other proportions; and I find it convenient to adjust these proportions in accordance with the top temperature and  $\text{CO}_2$  ratio in the top gas, increasing the proportion of hot gas withdrawn with rise of top temperature and fall of  $\text{CO}_2$  ratio and vice versa. I may thus hold the top temperature and  $\text{CO}_2$  ratio at a desired point, corresponding to a desired degree of utilization in the furnace of the fuel energy. Beyond a certain limit, the greater the proportion of hot gas taken from the furnace at 21, the smaller the proportion of the fuel energy utilized in the furnace and hence, the application of electric heat remaining sufficient to balance losses, the greater the consumption of carbon per pound cyanid. For example, with a hot gas withdrawal of about 58 per cent with 42 per cent of the gases from the combustion zone rising through the shaft and passing out of the furnace through 23 (together with gases formed in the shaft), the work devolving upon the combustion zone is about the equivalent of steps (2) and (3). With electric heat compensating heat losses in the combustion zone, this work requires the gasification of about 0.49 pound carbon (preheated to  $1200^\circ$ ) with air at  $750^\circ$ . An equation for the reaction might be written:



Upon this equation a statement can be based, the statement that the reaction between carbon, sodium oxid and air in these proportions (the carbon and soda being preheated 110 to  $1200^{\circ}$  and the air to  $750^{\circ}$ ) absorbs no heat and it follows that with air in greater proportions, or if the materials be more highly preheated the reaction is exothermic. Putting it in another way: The theoretical 115 temperature of the gasification of preheated carbon, 42 per cent by preheated soda and 58 per cent by air preheated to  $750^{\circ}$  is about  $1200^{\circ}$ . Some 13 per cent of the air nitrogen is fixed as cyanid vapor in a concentration of about 14 per cent of the products of the gasification. With cyanid recovered 120 from 58 per cent (by volume) of these products and the other 42 per cent being utilized for preheating more soda and carbon, the total consumption of carbon is about 1.17 pound per pound cyanid produced. The proportions of soda and fuel (90% carbon) charged into the furnace should in this case be about 45:55. It may be noted that in 125 130

any case these proportions should be carefully adjusted in correlation with the volume of hot gas withdrawn at 21 and the concentration of cyanid therein. Carbon 5 may be introduced into the hot zone of the furnace in the form of liquid or gaseous hydrocarbons in volume so regulated as to adjust the proportions of alkali and carbon as desired. By increasing the electric energy 10 applied the consumption of carbon may be reduced and a greater proportion of gas may be withdrawn through the hot gas outlet without reducing the concentration of cyanid in such gas. The regulation of the 15 furnace operation is a matter of coordinating the volume of hot gas withdrawn with the blast temperature and with the application of electric power, in conjunction with the proportions of alkali and carbon.

20 In applying the present invention to the general problem of nitrogen fixation, cyanid made as described is hydrolyzed to ammonia with recovery of alkali and this alkali may be returned to the furnace to be again 25 cyanided. It is advantageous to practise the invention in a blast furnace in simultaneously producing cyanid and iron or ferroalloy.

What I claim is:—

- 30 1. The process of making cyanid which comprises establishing and maintaining in a suitable reaction chamber a dominant mass or pool of cyanid in the liquid and vapor states, feeding cyanid forming materials into 35 said reaction chamber to react with said cyanid and maintaining the temperature and the predominance of cyanid in the reaction zone by aid of heat supplied by electrical means.
- 40 2. The process of making cyanids which comprises feeding air, alkali and carbon into a reaction chamber in which is maintained by aid of heat supplied by electrical means a mass of cyanized carbon at a temperature above 1000° C.
- 45 3. The process of making cyanids which comprises feeding air, alkali and carbon into a reaction chamber in which is maintained by aid of heat supplied by electrical means 50 a mass of cyanized carbon at a temperature above 1000° C. and removing cyanid from the sphere of reaction.
- 55 4. The process of making cyanids which comprises downwardly feeding air, alkali and carbon into a reaction chamber in which is maintained by aid of heat supplied by electrical means a mass of cyanized carbon at a temperature above 1000° C. and removing cyanid from the sphere of reaction.
- 60 5. The process of making cyanids which comprises downwardly feeding air, alkali and carbon into a reaction chamber in which is maintained by aid of heat supplied by electrical means a mass of cyanized carbon 65 at a temperature above 1000° C. and remov-

ing cyanid from the bottom of said reaction chamber.

6. The process of making cyanid which comprises contacting a mass of alkalinized carbon heated electrically to a cyanid forming temperature with a mass of nitrogen and oxygen so regulated that the proportion of cyanid and alkali in the resulting cyanized carbon is greater than the proportion of equivalent alkali in the initial alkalinized carbon. 75

7. A process of making cyanid which comprises contacting alkali vapor and nitrogen with cyanized carbon maintained at a temperature above 1000° C. with the aid of heat supplied by electrical means. 80

8. A process of making cyanid which comprises feeding alkali, carbon and nitrogen into a reaction chamber to react with a mass of cyanid therein maintained at a temperature above 1000° C., removing cyanid laden gases therefrom and quickly cooling said gases to deposit cyanid substantially without reversion. 85

9. A process of making cyanid which comprises passing nitrogen into contact with alkali and carbon maintained at a cyanid forming temperature and quickly cooling resulting gases to deposit cyanid therefrom substantially without reversion. 90

10. A process of making sodium cyanid which comprises heating together to a cyanid-vapor-forming temperature sodium carbonate, carbon and nitrogen and quickly cooling resulting gases to deposit sodium cyanid substantially without reversion. 100

11. A process of making cyanid which comprises contacting nitrogen with alkali and carbon at a cyanid forming temperature maintained with aid of heat supplied to the sphere of reaction by means of electrical currents induced therein or in proximity thereto. 105

12. In nitrogen fixation the process which comprises contacting air preheated to substantially above 500° C., with alkalinized and cyanized charcoal maintained at about 1200° C., by aid of heat supplied by electrical means. 110

13. In the manufacture of cyanids the process which comprises contacting at a temperature above 1000° C., preheated carbon and alkali under gas producing conditions with preheated air, recovering cyanid from a regulated proportion of the gases produced while preheating carbon and alkali with another regulated portion of said gases, and maintaining the temperature and a substantial concentration of cyanid vapor in the gases by aid of heat supplied by electrical means. 115

14. In the manufacture of sodium cyanid the process which comprises contacting at cyanid-vapor-forming temperatures preheated carbon and soda under gas producing 120

conditions with preheated air, recovering sodium cyanid from a regulated proportion of the gases produced while preheating carbon and soda with another regulated portion of said gases, and maintaining the temperature and a substantial concentration of cyanid vapor in the gases by aid of heat supplied by electrical means.

15. In cyanid making the process of cooling hot cyanid laden gases and depositing cyanid therefrom substantially without reversion which comprises leading such gases into a cooling chamber in which a relatively large mass of cooled gas is maintained.

16. The process of making sodium cyanid which comprises feeding nitrogen, soda and carbon into a reaction chamber in which is maintained by aid of heat supplied by electrical means a mass of cyanized carbon at a

20 temperature above 1000° C.

17. In making cyanid vapor by heating together in a shaft furnace carbon, alkali and air in the presence of cyanid, the process of providing in the hot zone a volume 25 of heat available for work at cyanid forming temperatures which comprises reinforcing by heat electrically supplied the heat developed by CO formation from preheated air and carbon preheated by counter-current contact in the shaft with a regulated pro-

portion of cyanid-laden gases previously produced.

18. In the fixation in a blast furnace of nitrogen as cyanid vapor by gasifying carbon with soda and air at temperatures above 35 1000° C., the process of making the cyanid forming reaction exothermic which comprises regulating the relative proportions of alkali and carbon charged into the furnace in correlation with the blast heat and 40 preheating said carbon and soda by counter-current contact in the furnace shaft with a regulated proportion of the cyanid-laden gases produced in the hearth, cyanid being recovered by quickly cooling another portion 45 of such gases withdrawn from the furnace at a level of high temperature.

19. In making cyanid from carbon, alkali and nitrogen in the presence of preformed cyanid in a shaft furnace heated by electrical means, the process of controlling the heat economy of the operation which comprises preheating the carbon and alkali descending through the furnace shaft to the electrically-heated zone by counter current contact 50 55 with a regulated quantity of ascending cyanid-laden gases.

In testimony whereof, I have hereunto affixed my signature.

K. P. McELROY.